

# UNITED STATES PATENT OFFICE.

JAMES C. FITZSIMMONS, OF SAN FRANCISCO, CALIFORNIA.

## WOOD-PRESERVATIVE.

1,111,302.

Specification of Letters Patent. Patented Sept. 22, 1914.

No Drawing.

Application filed June 23, 1913. Serial No. 775,814.

*To all whom it may concern:*

Be it known that I, JAMES C. FITZSIMMONS, a citizen of the United States, residing in the city and county of San Francisco, and State of California, have invented new and useful Improvements in Wood-Preservatives, of which the following is a specification.

This invention relates to wood preservatives and pertains especially to means for preserving piling and other timbers from the attack of the teredo and other marine insects.

The decay of wood takes place owing to the presence of living germs, fungi, or bacteria. These germs attack the cellulose and lignin of the wood cells, which serve as a food for their development. Moisture, heat and air are also necessary for their development. The heat of almost any climate is sufficient. So heat and air are beyond practical control.

A preservative for wood must therefore have the following qualities: 1.—Antiseptic, or capable of killing hostile germs. 2.—Able to exclude such germs. 3.—Able to exclude air and moisture.

I have found a very satisfactory and serviceable preservative in a mixture of heavy mineral oil of asphaltic base and approximately 14° Baumé gravity, such as is produced in quantity in California, and cresylic acid (cresol) of approximately 97% pure.

Cresylic acid is a very active antiseptic and is preferred for many reasons: 1st.—Its specific gravity (.98) is about the same as the heavy California oil (.96 such as I prefer), so that the resulting mixture is practically stable. 2nd.—Like heavy oil it has a fairly high boiling point; thus allowing the mixture to be heated to the desired degree for most advantageous application without any loss by volatilization of the antiseptic properties. 3.—It is readily miscible with the asphalt of the oil and the asphaltic derivatives and the mixture is water-proof. The metallic salts which are antiseptic do not readily mix with asphaltum, but deposit on or in the wood as crystals which are easily soluble.

The proportions of the mixture are approximately 90% to 95% heavy oil, and 10% to 5% cresylic acid. The mixture is made

at a temperature of approximately 150° F.; the oil being first heated and the cresylic acid then added and stirred until complete admixture takes place. The preservative is applied hot (approximately 150° to 200° F.) either as a paint or by immersion of the wood to be treated in a vat containing the heated mixture or in any other suitable manner.

This preservative is advantageous for many reasons: The asphalt or other base of the oil will fill the cells and pores of the wood and exclude moisture, air and germs. They are non-volatile and do not crystallize as naphthalene does in creosote. It is insoluble in water and most chemicals. Has a high-melting point and will not exude under climatic conditions. It can be standardized and always available as a standard product. The components are obtainable in the markets of the world, at reasonable prices. The components and mixture can be readily handled with safety and with simple apparatus. The mixture can be controlled so that no "bleeding" or exudation from the wood occurs. After processing the wood is immediately available for service.

Having thus described my invention what I claim and desire to secure by Letters Patent is:—

1. A wood preservative consisting of a mixture of heavy mineral oil and cresol.
2. A wood preservative consisting of a mixture of oil of asphaltum base of approximately 14° Baumé with approximately 10 per cent. of cresol.
3. A wood preservative consisting of a mixture of oil of asphaltum base of approximately 14° Baumé with approximately 10 per cent. of cresol and having a boiling point of about 200° centigrade.

4. A wood preservative consisting of a mixture of heavy mineral oil having a specific gravity approximately .98 and cresol having substantially the same specific gravity.

In testimony whereof I have hereunto set my hand in the presence of two subscribing witnesses.

JAMES C. FITZSIMMONS.

Witnesses:

JAMES K. FIRTH,  
T. LAMMON.